

Nov. 14, 1939.

L. C. JONES ET AL

2,179,790

PHOTOGRAPHIC DEVELOPER

Filed June 14, 1939

2 Sheets-Sheet 1

**FIG. 1.**

**DK-50 TYPE DEVELOPER**



INVENTORS  
LOUIS C. JONES  
ROBERT BOWLING BARNES,  
BY GARNET PHILIP HAM,

*Robert B. Barnes*  
ATTORNEY.

Nov. 14, 1939.

L. C. JONES ET AL

2,179,790

PHOTOGRAPHIC DEVELOPER

Filed June 14, 1939

2 Sheets-Sheet 2

**FIG. 2.**

**DK-60 TYPE DEVELOPER**



INVENTORS  
LOUIS C. JONES,  
ROBERT BOWLING BARNES,  
BY GARNET PHILIP HAAS  
Robert James Martin  
ATTORNEY.

## UNITED STATES PATENT OFFICE

2,179,790

## PHOTOGRAPHIC DEVELOPER

Louis C. Jones, Greenwich, Robert Bowling Barnes, Stamford, and Garnet Philip Ham, Old Greenwich, Conn., assignors to American Cyanamid Company, New York, N. Y., a corporation of Maine

Application June 14, 1939, Serial No. 279,094

14 Claims. (Cl. 95—88)

This invention relates to photographic developers, and more particularly to developers for photographic negatives which are capable of variation of contrast.

5 This application is a continuation in part of our application Ser. No. 218,972, filed July 13, 1938, and now Pat. No. 2,165,797, July 11, 1939.

The ordinary type of photographic developer of which the metol-hydroquinone types are the most 10 common normally contain at least three types of ingredients; the actual developers such as metol, hydroquinone and the like, protective agents against oxidation such as sodium sulfite, and a suitable alkali to produce a pH suited for 15 the particular developer. In addition, other ingredients such as restrainers, for example alkali metal bromides and in the case of tropical developers, sodium sulfate, may be present. Normally, a developer formula is balanced with regard to the three main ingredients in order to 20 give results and produce a satisfactory fidelity in reproducing the various gradations of light and shadow of the object photographed. When a curve is constructed having ordinates proportional to the density of the final developed negative, that is to say, the negative logarithm of 25 transmission and with abscissae proportional to the logarithm of exposure, there should be a long, reasonably straight portion of the curve in order to reproduce with reasonable fidelity 30 various exposures within a certain range. With most modern developers, satisfactory fidelity is obtained, but a relatively large number of formulae are in use because it is difficult to change 35 the characteristics of a particular formula without upsetting its balance.

A few years ago, a new alkali consisting of a mixture of alkaline substances, notably borates, was introduced by the Eastman Kodak Company under the name "Kodalk" and is covered by U. S. 40 Patent No. 1,990,800. Four different formulae of the Eastman Kodak Company, namely DK-15, DK-50, DK-60 and DK-76, have been formulated using the new alkali and claims have been made 45 for "Kodalk" that contrast can be varied within wide limits by variation in the amount of alkali without upsetting the balance of the developer, thus producing results which give poor fidelity. This is an important advantage as it makes possible 50 the use of a relatively small number of formulae for a wide number of purposes since it is possible to vary the contrast within considerable limits by variation of the alkali component without requiring a complete recalculation of the 55 entire formula.

While "Kodalk" possesses the properties claimed for it to a considerable degree and thus represents a distinct advance over the use of standard alkalies such as sodium carbonate, in some formulae it leaves much to be desired. Its change in contrast is sometimes accompanied by a loss of fidelity. According to the present invention, it has been found that a new class of bases which can be used to supply the alkaline reaction necessary for most photographic developers possesses the advantages of variation in contrast with variation in amount of the base, and in some formulae the best of them are superior in this respect to "Kodalk". The compounds of the present invention are quaternary 10 ammonium hydroxides which are strong organic bases. Among the most effective compounds of the present invention are trimethylbenzylammonium hydroxide, known to the trade as "Tetone B", and tetramethylammonium hydroxide. 15

The invention will be described in detail in conjunction with specific examples illustrating the use of the compounds of the present invention in typical metol-hydroquinone developer formulae. The compounds are also useful in other types of developers such as those using p-phenylene diamine and Glycine, but are of less importance with this class of developers which are normally used at low contrast to produce extreme fine grain. The invention will also be described in conjunction with curves showing the results of densitometric measurements on exposed negatives which are illustrated on the drawings in which 20

Fig. 1 represents a series of curves with a DK-50 type developer; and

Fig. 2 is a series of curves with a DK-60 type developer.

Example 1

|                      |       |       |    |
|----------------------|-------|-------|----|
| Water                | cc.   | 500   | 40 |
| Metol                | grams | 1.25  |    |
| Sodium sulfite, des. | do    | 15.00 |    |
| Hydroquinone         | do    | 1.25  | 45 |
| "Kodalk"             | do    | 5.00  |    |
| Potassium bromide    | do    | 0.25  |    |

This formula DK-50 is one used for the development of normal films of both orthochromatic and panchromatic type.

Two developers were prepared according to the Eastman Kodak DK-50 formula as follows, the first having five times the normal amount of "Kodalk" and the second having an amount of 55

trimethylbenzylammonium hydroxide to give the same pH as the first:

A photographic wedge made by the Eastman Kodak Company and having nine steps between light and dark arranged logarithmically, each step from dark to light representing a transmission 150% that of the preceding step, was used to make exposures on 35 mm. Eastman Kodak Supersensitive panchromatic film. This film was chosen as being representative of a medium fast, long latitude panchromatic film which would show up lack of fidelity or excessive fogging rapidly and which is a type of film where variations in contrast produced by the developer are normally most necessary. All exposures were carefully calibrated using a Leitz enlarger with a 10 watt bulb and lens stopped down to F12.5 as a source of illumination. All conditions of development including time, temperature, agitation, fixing, washing and the like were kept uniform and the only difference between the tests was the developer used. Densitometric measurements were made in a photoelectric densitometer calibrated against the wedge used for the exposures. The densitometric readings are plotted in the curves shown in Fig. 1. It will be noted that trimethylbenzylammonium hydroxide gave results similar to the "Kodalk" with slightly less contrast but greater fidelity as evidenced by the longer more perfectly straight portion of the curve.

#### Example 2

A developer was prepared according to the Eastman Kodak DK-50 formula having an amount of tetramethylammonium hydroxide to give a pH of the same value as the developer of Example 1 containing five times normal "Kodalk". A photographic wedge was prepared as in Example 1 and a curve of the densitometer readings is also shown in Fig. 1. Examination of the curve indicates better fidelity and only slightly less contrast than the "Kodalk" curve.

#### Example 3

45 A surprising result is obtained when mixtures of trimethylbenzylammonium hydroxide and sodium carbonate are used. The mixtures appear to have substantially the desirable characteristics of the quaternary ammonium hydroxide alone.

The formula DK-50 type was prepared substituting a mixture of 3.82 cc. of trimethylbenzylammonium hydroxide and 5.10 grams of sodium carbonate to produce a five times concentrated developer. The pH was approximately 10.65. A photographic wedge was prepared as in Example 1 and a curve of the densitometer is shown in Fig. 1. It will be noted as shown by the curves of Fig. 1 that this mixture produced a curve having better contrast and equivalent fidelity to the "Kodalk". The possibility of substituting sodium carbonate for a considerable part of the quaternary ammonium compound represents a real commercial advantage because of the lower price of the sodium carbonate.

#### Example 4

|                     |       |       |
|---------------------|-------|-------|
| Water               | cc    | 500   |
| Metol               | grams | 1.25  |
| Sodium sulfite, des | do    | 15.00 |
| Hydroquinone        | do    | 1.25  |
| "Kodalk"            | do    | 10.00 |
| Potassium bromide   | do    | 0.25  |

This type developer DK-60 is also intended for general development of films of both the orthochromatic and panchromatic type where a somewhat higher contrast is desired.

Two developers were prepared according to the Eastman Kodak formula DK-60 as follows, the first containing five times the amount of "Kodalk" and the other an amount of trimethylbenzylammonium hydroxide to give an equivalent pH. Photographic wedges were prepared as in Example 1 and densitometer readings were taken and plotted into curves as shown in Fig. 2.

It will be noted that the contrast and the fidelity are somewhat better than that of "Kodalk".

What we claim is:

1. A photographic developer for silver halides containing as an alkalinity producing agent a quaternary ammonium hydroxide in effective amount.
2. A photographic developer for silver halide containing as the sole alkalinity producing agent a quaternary ammonium hydroxide.
3. A metol-hydroquinone photographic developer containing as an alkalinity producing agent a quaternary ammonium hydroxide in effective amount.
4. A metol-hydroquinone photographic developer containing as the sole alkalinity producing agent a quaternary ammonium hydroxide.

5. A photographic developer for silver halides containing as its alkalinity producing agent a mixture of sodium carbonate and a quaternary ammonium hydroxide in effective amounts.

6. A metol-hydroquinone photographic developer containing as its alkalinity producing agent a mixture of sodium carbonate and a quaternary ammonium hydroxide in effective amounts.

7. A photographic developer for silver halides containing as its alkalinity producing agent tetramethylammonium hydroxide in effective amount.

8. A metol-hydroquinone photographic developer containing as its alkalinity producing agent tetramethylammonium hydroxide in effective amount.

9. A photographic developer for silver halides containing as its alkalinity producing agent a mixture of sodium carbonate and tetramethylammonium hydroxide in effective amounts.

10. A metol-hydroquinone photographic developer containing as its alkalinity producing agent a mixture of sodium carbonate and tetramethylammonium hydroxide in effective amounts.

11. A photographic developer for silver halides containing as its alkalinity producing agent trimethylbenzylammonium hydroxide in effective amount.

12. A metol-hydroquinone photographic developer containing as its alkalinity producing agent trimethylbenzylammonium hydroxide in effective amount.

13. A photographic developer for silver halides containing as its alkalinity producing agent a mixture of sodium carbonate and trimethylbenzylammonium hydroxide in effective amounts.

14. A metol-hydroquinone photographic developer containing as its alkalinity producing agent a mixture of sodium carbonate and trimethylbenzylammonium hydroxide in effective amounts.

LOUIS C. JONES.

ROBERT BOWLING BARNES.

GARNET PHILIP HAM.